

F. D. S. ROBERTSON.

PROCESS FOR RECOVERING MOLYBDENUM FROM ITS ORES AND CONCENTRATES.

APPLICATION FILED NOV. 14, 1913.

1,118,150.

Patented Nov. 24, 1914.

2 SHEETS-SHEET 1.



Fig. 4

Fig. 5

Fig. 6



Fig. 1

WITNESSES

J. P. Bradley  
F. F. Bradley

INVENTOR

F. D. S. Robertson  
Inventor

F. D. S. ROBERTSON.

PROCESS FOR RECOVERING MOLYBDENUM FROM ITS ORES AND CONCENTRATES.

APPLICATION FILED NOV. 14, 1913.

1,118,150.

Patented Nov. 24, 1914.

2 SHEETS-SHEET 2.



WITNESSES

J. P. Brody  
F. L. Boothby

INVENTOR  
Frederick D. S. Robertson  
H. C. Davis & Associates  
Assessors

# UNITED STATES PATENT OFFICE.

FREDERICK D. S. ROBERTSON, OF TORONTO, ONTARIO, CANADA, ASSIGNOR OF THREE-FOURTHS TO MICHAEL J. O'BRIEN, OF RENFREW, ONTARIO, CANADA.

## PROCESS FOR RECOVERING MOLYBDENUM FROM ITS ORES AND CONCENTRATES.

1,118,150.

Specification of Letters Patent.

Patented Nov. 24, 1914.

Application filed November 14, 1913. Serial No. 800,981.

To all whom it may concern:

Be it known that I, FREDERICK DUNCAN STRUAN ROBERTSON, a subject of the King of Great Britain, and resident of the city of Toronto, in the county of York and Province of Ontario, Dominion of Canada, have invented a new and useful Process for Recovering Molybdenum from its Ores and Concentrates; and I hereby declare that the following is a full, clear, and exact description of the same.

The process is applicable generally to such of the rare metals as form at least one volatile oxid, and is of particular value for the production by volatilizing-roasting, and subsequent condensation, of the tri- or molybdcic and other oxids of molybdenum directly from its ores and concentrates.

Of the various oxids of molybdenum it is most desirable to form the tri- or molybdcic oxid,  $MoO_3$ , which melts at a temperature of about  $790^{\circ}$  Cen. This is accomplished by maintaining a temperature of about  $800^{\circ}$  Cen. with excess of oxygen, according to the reaction:—



with the formation of fine silky acicular crystals of a very volatile character and readily sublimed. Under these conditions of temperature and atmosphere the tri-oxid of molybdenum,  $MoO_3$ , is alone produced, the operation being materially hastened with the addition of steam, thus:—



The process will therefore be hereinafter described as applied to the production particularly of the tri-oxid of molybdenum from ores or concentrates containing molybdenum by a direct process of volatilizing-roasting in a highly oxidizing atmosphere, this being the essential feature of the present invention.

The ores, concentrates, middlings and tailings, containing molybdenum, which will hereafter for convenience be called ores, are crushed, preferably through rolls in order to preserve the flakes and thus expose a greater surface to oxidizing influences, to about eight mesh and introduced to a suitable furnace, muffle or retort.

The type of apparatus by which the process may be carried into practice is purely

arbitrary, but for the purpose of describing the various steps a conventional type of plant is shown in which—

Figure 1, is a longitudinal section of a rotary furnace, Fig. 2, is a longitudinal section of the cooling tower and bag house, Fig. 3 is a cross-section of the furnace, and Fig. 4 is a broken detail view of the twyered air and steam pipes.

In Fig. 1, *a* is the roasting cylinder, *b*, the ore hopper arranged so as to continuously deliver the ore into the roasting cylinder from which it drops out in its spent condition into the chamber *c*, from which it is delivered into the truck *d*. The fireplace is in the chamber *f*, which may either be within or at the side of the chamber *c*. Longitudinal ribs *a'* projecting from the lining of the furnace *a* raise the powdered ore as the furnace rotates, and allow it to fall through the heated gases as soon as its angle of repose is exceeded. The fumes and gases pass out at the upper end of the furnace into the cooling chamber *g*, and thence through the flue *o* to the dust tower *p*, and bag-house or filter-chamber *t*, (Fig. 2).

In addition to the air which enters through the firing door of the fire chamber *f*, a further supply of air under a pressure of about five pounds per square inch, which has been previously pre-heated by passing through the cooling chamber *g*, is maintained by means of the twyered pipe *m*, the air being moistened by steam which enters through the branched pipe *n*.

Different degrees of inclination, to suit different ores and concentrates, can be given to the furnace. During the passage of the fumes through the cooling chamber *g*, which may be divided into water-cooled compartments *g'*, and is preferably built of solid masonry, considerable condensation takes place, the crystals being withdrawn at intervals through the ports *h*. After their passage through the cooling chamber *g*, the fumes and gases are drawn through the flue *o* into the dust tower *p*, see Fig. 2, by means of the fan *s* placed behind it. Several towers may be employed, and in series, and they may also contain partition walls.

From the last dust tower the gaseous fume current is drawn off by the fan *s* into the main *r* connected with the distributing main *k* which runs the whole length of the

bag-house or filter-chamber *t*. There may be a series of mains *k* near the roof of the bag-house and from which, at intervals of about three feet, branch pipes *j*, project, to each of which are connected bags *l* made of strong cotton or preferably wool about thirty to forty feet long, and about two feet in diameter. These bags may be either open at their lower end and thus connect with casks or bins, or be connected at the bottom in a U-shape. The fine oxid of molybdenum collects inside these bags, while the permanent gases, sulfur dioxide, etc., passing through the meshes of the fabric are drawn off by the fan *v*, and are led into the open stack *x*. The waste gases may be recovered to form sulfuric and other compounds, and their heat may be utilized toward raising steam. The charge having thus been introduced into the furnace, the temperature is steadily maintained together with a plentiful oxidizing current, otherwise oxids other than the tri-oxid of molybdenum are apt to be formed and in which case the mass tends to frit and present a frozen appearance. The action of pre-heated air under pressure together with steam and also occasional fresh additions of ore or concentrates will, however, overcome this obstacle. During the roast the charge should present a reddish appearance and should feel somewhat soft under the rabble, but should not be allowed to become tacky. In order that the charge remain in a more or less pulverulent state and thus permit of a free access of air, it may be necessary to mix with it crushed quartz or sand, but such additions must be carefully added, the character of the ore being taken into account as the resulting mixture may react too strongly upon the furnace lining. A similar effect may also be produced, especially in

the case of highly pyritic ores, by a suitable addition of lime or other alkaline earth, this having the further benefit of a desulfurizing agent which absorbs much of the sulfur content. 45

Properly roasted ore should possess an ashy gray color on cooling, and the actual roasting period may take three or four hours 50 according to the character of the ore or concentrate.

The temperature in the bag-house must not exceed 120° Cen. when woolen bags are used, or 90° when cotton bags are used. 55 Woolen bags are more efficient and last much longer than cotton; the bags are usually cleaned or shaken twice in twenty-four hours. The tri-oxid of molybdenum thus prepared is very pure, and may be further 60 purified, if desired, by similar re-sublimation in a separate similar plant.

Having now particularly described and ascertained the nature of the process and the manner of its performance, I now claim: 65

1. The direct process for the volatilization and recovery of molybdenum in the form of pure molybdenum trioxid  $\text{MoO}_3$ , which consists in subjecting ores containing molybdenum to a temperature exceeding 70 790 degrees centigrade in an atmosphere having an excess of oxygen.

2. The direct process for the volatilization and recovery of molybdenum in the form of pure molybdenum trioxid  $\text{MoO}_3$ , which consists in subjecting ores containing molybdenum to a volatilizing temperature, in an atmosphere having an excess of oxygen. 75

Toronto, Ont., November 10th, 1913.

FREDERICK D. S. ROBERTSON.

Signed in the presence of—

CHAS. H. RICHES,  
C. W. ADAMS.